

## UNITED STATES PATENT OFFICE

DONALD MCKNIGHT HEPBURN, OF PHILADELPHIA, PENNSYLVANIA, ASSIGNOR TO  
AMIESITE ASPHALT COMPANY OF AMERICA, OF PHILADELPHIA, PENNSYLVANIA,  
A CORPORATION OF NEW JERSEY

## BITUMEN ROAD PAVING

No Drawing.

Application filed March 31, 1927. Serial No. 180,075.

This invention relates primarily to improvements in that class of pavement or road surface employing a graded and bitumen-coated stone aggregate free from fines and 5 other void-filling elements and in which the aggregate is bonded and stabilized entirely by the bitumen coating of the individual stones.

More particularly the invention relates to 10 improvements in the pavement forming the subject of my U. S. Patent No. 1,611,444, issued December 21, 1926; and it is the principal object of the present invention to provide means whereby a thicker and stronger 15 coating of bituminous substance, such as asphalt, may be made to adhere to the surfaces of the stones of the aggregate which results in a remarkable improvement in the finished pavement, as hereinafter set forth.

20 I have found in practice that the fracture surfaces of different types of stone vary largely in character. In some cases the surfaces are comparatively smooth, while other stones give extremely rough surfaces. In 25 building roads of the above mentioned type, and where the aforesaid rough surfaces are met with, I have found it particularly desirable, if not essential, in order to properly bond the aggregate and cement the individual stones together, to provide a thicker 30 and stronger coating of asphalt or other bitumen than would normally be required where the fracture is cleaner or than can be obtained by the usual methods. This will be 35 understood when it is stated that for a maximum cementing effect between two objects all the recesses between and in the abutting surfaces of the objects should be filled by the cementing medium.

40 I have discovered, in the present instance, that the bonding and cementing coating on the surfaces of the stones of the aggregate may be materially increased in thickness and improved in character by making a mortar 45 of the bituminous cementing medium which is accomplished by adding thereto and thoroughly incorporating a predetermined quantity of sand, or clean, crushed rock screenings, or the like. In general, I prefer to use 50 from four to eight per cent by weight of the sand or rock screenings for any given amount of bitumen, although the amounts may vary beyond these limits in special cases. By this means I have found it possible to hold from five to seven per cent, and even more, asphalt 55 cement on the surfaces of the stone than is possible using the asphalt or other bitumen unmixed with the sand, screenings or equivalent material. The bitumen mortar does not run on the stone surfaces; the aggregate does 60 not settle in the mixture in shipment; and the unloading and handling qualities of the paving mixture remains unaffected.

In practicing the present invention, I may 65 coat the stone in accordance with the procedure outlined in the aforesaid Patent No. 1,611,444, but using a larger amount of the bitumen as compared with quantity of aggregate to be coated. Following the thorough 70 mixing of the bitumen with the stone the sand or screenings is added and the mixing operation continued until the added material is thoroughly incorporated. The sand, 75 screenings or the like has the effect of strengthening the bitumen coating and permits of a greater amount adhering to the surfaces without running. While I prefer to add the sand or like material after the stones have been thoroughly coated with the bitumen, it is possible without departure from 80 the invention to incorporate the sand in the bitumen prior to the addition of the latter to the aggregate. Or the bitumen and sand may be simultaneously mixed with aggregate. The stone sizes of the aggregate and the 85 method of laying the composition may also be in accordance with the procedure set forth in the patent.

It will be noted that I depend entirely on 90 an aggregate of crushed stone with the fines under a given size removed so that my pavement is composed entirely of dust free stone. When the mixture is rolled into place and compacted, the particles of the aggregate or 95 pieces of stones lie in close contact with each other, like a piece of masonry, and the voids between the stones are not filled with fine aggregate. The separate pieces of stone in the aggregate are pushed and wedged together, however, in as intimate a relation as it is 100

possible to get them. The road depends for cohesion and stability entirely on the bonding effect of bitumen with which the stone is coated, and it is important that the cementing medium be adequate for all the varying types of aggregate that may be used. In order that I may properly cement, for example, two very rough surfaces together with a bitumen cement so that the surfaces are properly filled as described above, I must have a heavy coating of bitumen cement on each individual piece of stone. The heavy, strong coating of bitumen provided by the present invention meets these requirements.

16 It should be further noted that my pavement is strictly a bitumen cemented road in which the design has been carefully worked out to produce voids in the pavement in order to establish innumerable expansion joints, 20 and establish a pavement that is flexible and can move without cracking with the expansion and contraction that takes place in the earth's surface. It is therefore essential that the bitumen and sand content be kept within 25 the amount that can be held on the stone surfaces without excess and without filling the voids. With the addition of sand or clean stone screenings preferably added to the mixture just after the asphalt has been 30 properly distributed on the stone particles a mortar is produced increasing the thickness of the bitumen cement to such an extent that I can hold from five per cent (5%) to ten per cent (10%) more asphalt on the stone 35 surfaces and produce a tighter bond and an improved material in sealing qualities without appreciably reducing the voids in my pavement or reducing the non-skid qualities of my pavement.

40 In practice, I have noted a marked improvement in roads made with stone aggregate coated in accordance with my invention; and this improvement is noted not only in the type of pavement constructed, as described, 45 with unfilled voids, but in all pavements employing a bitumen coated aggregate.

It will be understood that the word sand used in the claim is comprehensive of fine rock screenings and other relatively fine 50 mineral particles.

I claim:

55 A method of making a bituminous concrete for open pavements, which consists in coating a mineral aggregate comprising clean, graded, broken stone, with a bituminous cement in a fluent, mobile condition by thoroughly agitating said aggregate in the presence of said fluid cement, the quantity of cement so admixed with the aggregate being 60 substantially greater than what would remain on the aggregate were said agitation to cease, and then adding to said mobile cement on said aggregate still under agitation a quantity of clean, sandy fines insufficient to appreciably 65 reduce the voids in the finished pavement,

but sufficient to form on each piece of aggregate a thick, stable coating of cement and sand which will not run out of the mixture when said agitation is discontinued, but will remain permanently on and cover each of the individual pieces of aggregate at atmospheric temperatures and maintain said material sufficiently loose and friable to be handled and transported until it is compacted upon the roadway.

DONALD McKNIGHT HEPBURN.

70

75